

## UNITED STATES PATENT OFFICE

1,963,197

## COLOR PHOTOGRAPHY AND CINEMATOGRAPHY

Alfred Froehlich, Dessau in Arholt, Germany,  
assignor to Agfa Ansco Corporation, Binghamton, N. Y., a corporation of New York

No Drawing. Application May 16, 1932, Serial No. 611,757. In Germany May 16, 1931

8 Claims. (Cl. 95-2)

My present invention relates to color photography and cinematography.

One of its objects is to provide a process of converting pictures composed of a finely divided metal and more particularly silver pictures into dyestuff pictures especially such constituted by diazo dyestuffs. Further objects will be seen from the detailed specification following hereafter.

10 I have found that the silver salts of the diazotates, particularly of the antidiiazotates of the formula



are very sparingly soluble in water. By shaking, for instance, silver chloride with a diazotate solution, the silver compound can be converted 20 into silver diazotate, chlorine ions passing into solution.

This observation leads to the preparation of dyestuff pictures from pictures composed of a finely divided metal, more particularly silver pictures, produced in the usual photographic manner. The process of this invention consists in bleaching out, for instance, a silver picture to silver chloride by means of a solution of copper chloride or the like, treating the latter for some 30 minutes with a solution of a soluble antidiiazotate, alkali compounds being specially suitable to this end, washing out the excess of diazotate with water and coupling the silver diazotate which has been produced in the picture layer with an azo 35 dyestuff component to obtain an azo dyestuff of the shade desired in each special case.

The coupling process may be carried out in an acid or in an alkaline medium. Whereas it is realized very easily in an acid solution, it is advisable to accelerate the process, when working 40 in an alkaline medium, by heat and to use a previously hardened picture layer. After coupling the picture is washed for some minutes with water, whereafter the silver or silver salt which separates 45 in the coupling process and may still be present in the layer is extracted, in the usual manner, by means of a fixing bath or a solvent for the silver or salts thereof, so that a pure azo dyestuff picture is produced.

50 According to the process of this invention it is possible to obtain, by a suitable selection of the components, any desired tint, and particularly to produce the dyes which are best suited for purposes of the two- and three-color photography or cinematography. For the preparation of a two-

or three-color picture, the picture layers must be arranged on transparent or translucent supports, particularly on such as are made of a cellulose ester or regenerated cellulose, and the part-color pictures produced by printing the different part-color negatives according to the process described are brought into register as strictly as possible. If required, several picture layers may be arranged on a single support one over the other or on the two faces of the support, so that after printing it is not necessary to bring the part-pictures into registration. It is likewise possible to produce color pictures on an opaque support, for instance on paper. These pictures are viewed by reflected light.

70 Suitable antidiiazotates are, for instance, those of para-nitraniline,  $\beta$ -naphthylamine, benzidine, dianisidine, para-aminoazobenzene and a great many other compounds. As coupling components all components customary in the technique of manufacturing azo dyestuffs are suitable; those yielding dyestuffs insoluble in water are, however, preferred because the pictures produced thereby are particularly sharp. If the dyes are not sufficiently insoluble, their dissolution is prevented by adding to the solution containing the coupling component an agent having a salting-out action.

75 Coupling components which do not interact with or are not dissolved by photographic developing and fixing baths, may be incorporated in the metal halide emulsion more particularly the silver halide emulsion at some stage of the production of the emulsion. In this case it is possible to cover the support with superimposed layers of silver salt emulsions, containing different coupling components. If two coupling components are selected which form with the same diazo component in the one case a yellow and in the other case a purple dyestuff, it is possible to produce, by the use of suitably sensitized emulsions, on the one face of a support the yellow and the red part-picture, whereas the blue part-picture is produced on the other face of the support in a similar manner by means of a blue-coupling component. If during the coupling process a temperature higher than ordinary is used, the gelatin of the photographic layer is preferably hardened by means of formaldehyde or any other suitable hardening agent. The gelatin can be hardened at any stage in the production of the picture, but the hardening must precede the coupling process, thus the gelatin can be treated with a hardening agent during the production of the light-sensitive emulsion layer or after the pic-

60

65

70

75

80

85

90

95

100

105

110

ture composed of finely divided metal has been produced.

The following examples illustrate the invention:

5 *Example 1.*—A silver positive bleached out to silver chloride is placed for 10 minutes in a filtered solution of 1 gram of  $\alpha$ -naphthalene-sodium-antidiazotate dissolved in 100 cc. of water and containing an addition of a few drops of 10 caustic soda solution and is then washed for 45 minutes in running water. The picture now consists of  $\alpha$ -naphthalene-silver-antidiazotate, while the whites are free from diazotate. The picture is then immersed for 5 minutes in a solution of 15 2 per cent. strength of 1.8-diamino-naphthalene in sulfuric acid of  $1\frac{1}{2}$  per cent. strength, and washed with water. This operation may be followed, if desired, by a treatment in a thiosulfate bath in order to accelerate the dissolution of the 20 silver sulfate produced during the reaction, and by an after-treatment in water which has been slightly acidified. The picture obtained is blue.

25 *Example 2.*—A silver picture bleached out to silver chloride in gelatin hardened by means of formaldehyde is immersed for 10 minutes in a saturated solution of the antidiazotate of dianisidine which has been mixed with a small amount of caustic soda solution and filtered, and is then washed with water for one hour. For coupling, 30 the picture is treated with a solution of 1 per cent. strength of H-acid (1-amino-8-naphthol-3,6-disulfonic acid) heated to  $70^{\circ}$  C. After 1 to  $1\frac{1}{2}$  minutes the coupling process is complete. The picture is then well washed, the silver or 35 silver oxide which has been formed is bleached to silver chloride in a solution of cupric chloride, the silver chloride is dissolved in thiosulfate solution, and the picture is washed and subsequently bathed in slightly acidified water. The 40 picture obtained is likewise blue.

45 *Example 3.*—A silver chloride picture prepared according to Example 2 is bathed for 10 minutes in a solution of 1 per cent. strength of  $\alpha$ -naphthalene-antidiazotate which has been mixed with a small quantity of caustic soda solution and filtered; the picture is then rinsed with water and immersed for about 1 minute in a solution of 1 per cent. strength of H-acid of  $70^{\circ}$  C. The picture is washed in a solution of 2 per cent. strength 50 of potash alum. The bleaching and fixing baths according to Example 2 must also be mixed with potash alum in order to prevent bleeding. The picture obtained is red.

55 *Example 4.*—A picture of  $\alpha$ -naphthalene-silver-antidiazotate, prepared according to Example 3, is coupled with a resorcinol solution of 1 per cent. strength at  $70^{\circ}$  C. which has been saturated with sodium chloride. The picture is washed for a short time, bleached with cupric chloride, fixed 60 and washed again. The picture obtained is yellow.

65 *Example 5.*—The silver diazotate picture, prepared according to Example 3 is bathed for 5 minutes in an anthranilic acid solution containing sodium bicarbonate, and then dried. Coupling is effected by exposure for 2 minutes in a current of steam charged with a small amount of acetic acid. Then the picture is rinsed with water and fixed; it is orange.

70 *Example 6.*—The silver picture is converted, according to any of the known methods, into a silver halide picture and well rinsed with water. It is then bathed for 10 minutes in a saturated solution of  $\alpha$ -naphthalene-sodium-antidiazotate, 75 filtered, and mixed with some drops of caustic

soda solution. The picture is then rinsed with water for 1 hour. For coupling, the picture is dipped into a solution of 1-amino-8-naphthol-2,4-disulfonic acid to which some drops of acetic acid have been added. When operating at a temperature of  $40^{\circ}$  C. the coupling process is complete after 1 minute. After bleaching and fixing again a purple-red picture is obtained.

80 *Example 7.*—3.2 grams of  $\beta$ -naphthylamine are dissolved in alcohol to form a concentrated solution. The solution is added to 30 cc. of silver halide emulsion and the mixture cast on a plate of the size 18 x 24 cm. After exposure the plate is developed in the usual manner, fixed in a neutral fixing bath, washed, and bleached with a 2 per cent. solution of copper chloride. After having been washed, the plate is bathed for about 5 minutes in a cold solution of  $\beta$ -naphthyl-sodium-antidiazotate which has been made alkaline by a caustic alkali. Hereafter the plate is washed for about 30 minutes and the coupling process which sets in during this operation carried to an end in an acetic acid of 2 per cent. strength. After washing a red transparent diazo picture is obtained having clear whites.

85

90

95

100

What I claim is:

1. A dye-toning-process which comprises exposing to light a photographic material provided with an emulsion layer containing a light-sensitive silver halide, said silver being capable of forming a difficultly soluble diazotate, developing said exposed material, bleaching out the picture obtained and composed of finely divided silver, reacting on said bleached out picture with a diazotate, and treating the formed diazotate with a coupling compound.

105

2. A dye-toning-process which comprises exposing to light a photographic material provided with an emulsion layer containing a light-sensitive silver halide, said silver being capable of forming a difficultly soluble diazotate and a coupling compound, said coupling compound being not affected by the photographic developing baths, developing said exposed material, bleaching out the picture obtained composed of finely divided silver, reacting on said bleached out picture with a diazotate, and causing said coupling compound contained in the emulsion to interact with the formed diazotate.

115

3. A dye-toning-process which comprises exposing to light a photographic material provided with an emulsion layer containing a silver halide, developing said exposed material, bleaching out the silver picture obtained, reacting on said bleached out picture with an antidiazotate, and treating the formed silver antidiazotate with a coupling compound.

120

4. A dye-toning-process which comprises exposing to light a photographic material provided with an emulsion layer containing a silver halide and a coupling compound, said coupling compound being not affected by the photographic developing baths, developing said exposed material, bleaching out the silver picture obtained, reacting on said bleached out picture with an antidiazotate and causing said coupling compound contained in the emulsion to interact with the formed silver antidiazotate.

125

5. A dye-toning-process which comprises exposing to light a photographic material provided with several emulsion layers containing a silver halide and each layer being provided with a different coupling compound, said coupling compounds being not affected by the photographic developing baths, developing said exposed mate-

130

135

140

145

150

- rial, bleaching out the silver pictures obtained, reacting on said bleached out pictures with an antidiiazotate and causing said coupling compounds contained in the different emulsion layers to interact with the formed silver antidiiazotates. 5
6. A dye-toning-process which comprises exposing to light a photographic material provided with an emulsion layer containing a silver halide, developing said exposed material, bleaching out 10 the silver picture obtained, reacting on said bleached out silver picture for 10 minutes with a solution of 1 gram of  $\alpha$ -naphthalene-sodium-antidiiazotate in 100 cc. of water and containing an addition of some drops of caustic soda solution, washing the formed silver diazotate and 15 treating the diazotate for 5 minutes with a 2 per cent. solution of 1.8-diaminonaphthalene in sulfuric acid of  $1\frac{1}{2}$  per cent strength.
7. A dye-toning-process which comprises exposing to light a photographic material provided 20 with an emulsion layer containing a silver halide, developing said exposed material, treating the silver picture obtained with a hardening agent, bleaching out the silver picture contained in the hardened gelatin, bathing said bleached out picture in a saturated solution of the antidiiazotate 80 of dianisidine to which a small amount of caustic soda solution has been added, washing the formed silver diazotate, and treating the diazotate with a 1 per cent solution of H-acid heated to  $70^{\circ}\text{C}$ .
8. A dye-toning-process which comprises exposing to light a photographic material provided with an emulsion layer containing a silver halide and  $\beta$ -naphthylamine, developing said exposed material, fixing said material in a neutral fixing bath, bleaching out the silver picture obtained, reacting on said bleached out picture with  $\beta$ -naphthyl-sodium-antidiiazotate, and causing said  $\beta$ -naphthylamine contained in the emulsion to interact with the formed silver antidiiazotate. 85
9. A dye-toning-process which comprises exposing to light a photographic material provided with an emulsion layer containing a silver halide and  $\beta$ -naphthylamine, developing said exposed material, fixing said material in a neutral fixing bath, bleaching out the silver picture obtained, reacting on said bleached out picture with  $\beta$ -naphthyl-sodium-antidiiazotate, and causing said  $\beta$ -naphthylamine contained in the emulsion to interact with the formed silver antidiiazotate. 90
10. A dye-toning-process which comprises exposing to light a photographic material provided with an emulsion layer containing a silver halide and  $\beta$ -naphthylamine, developing said exposed material, fixing said material in a neutral fixing bath, bleaching out the silver picture obtained, reacting on said bleached out picture with  $\beta$ -naphthyl-sodium-antidiiazotate, and causing said  $\beta$ -naphthylamine contained in the emulsion to interact with the formed silver antidiiazotate. 95

ALFRED FROEHLICH.

|    |     |
|----|-----|
| 25 | 100 |
| 30 | 105 |
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |